



US007255901B2

(12) **United States Patent**  
**Yamaguchi et al.**

(10) **Patent No.:** **US 7,255,901 B2**  
(b5) **Date of Patent:** **Aug. 14, 2007**

(54) **RECORDING MEDIUM FOR INK AND METHOD FOR PRODUCING THE SAME**

(75) Inventors: **Kenichi Yamaguchi**, Chiba (JP); **Shigehira Iida**, Chiba (JP); **Tsuyoshi Santo**, Kanagawa (JP); **Yuji Kondo**, Tokyo (JP); **Motoaki Sato**, Tokyo (JP)

(73) Assignee: **Canon Kabushiki Kaisha**, Tokyo (JP)

(\*) Notice: Subject to any disclaimer, the term of this patent is extended or adjusted under 35 U.S.C. 154(b) by 0 days.

(21) Appl. No.: **10/678,143**

(22) Filed: **Oct. 6, 2003**

(65) **Prior Publication Data**

US 2004/0066446 A1 Apr. 8, 2004

**Related U.S. Application Data**

(63) Continuation of application No. PCT/JP03/07000, filed on Jun. 3, 2003.

(30) **Foreign Application Priority Data**

Jun. 4, 2002 (JP) ..... 2002-162910

(51) **Int. Cl.**

**B41M 5/50** (2006.01)

(52) **U.S. Cl.** ..... **428/32.3; 428/32.24; 428/32.25; 428/32.26; 428/32.29**

(58) **Field of Classification Search** ..... **428/32.25, 428/32.26, 32.3, 32.31**

See application file for complete search history.

(56) **References Cited**

**U.S. PATENT DOCUMENTS**

|             |         |                         |            |
|-------------|---------|-------------------------|------------|
| 4,202,870 A | 5/1980  | Weber et al. ....       | 423/630    |
| 4,242,271 A | 12/1980 | Weber et al. ....       | 260/448 AD |
| 4,248,852 A | 2/1981  | Wakabayashi et al. .... | 423/626    |
| 4,313,124 A | 1/1982  | Hara .....              | 346/140 R  |
| 4,345,262 A | 8/1982  | Shirato et al. ....     | 346/140 R  |

|             |        |                      |           |
|-------------|--------|----------------------|-----------|
| 4,463,359 A | 7/1984 | Ayata et al. ....    | 346/1.1   |
| 4,723,129 A | 2/1988 | Endo et al. ....     | 346/1.1   |
| 4,740,796 A | 4/1988 | Endo et al. ....     | 346/1.1   |
| 5,523,149 A | 6/1996 | Kijimuta et al. .... | 428/307.3 |
| 5,635,291 A | 6/1997 | Yoshino et al. ....  | 428/304.4 |
| 5,670,242 A | 9/1997 | Asano et al. ....    | 428/212   |
| 5,952,051 A | 9/1999 | Asano et al. ....    | 427/362   |

(Continued)

**FOREIGN PATENT DOCUMENTS**

EP 1 048 479 A2 11/2000

(Continued)

*Primary Examiner*—Pamela R. Schwartz

(74) *Attorney, Agent, or Firm*—Fitzpatrick, Cella, Harper & Scinto

(57) **ABSTRACT**

A recording medium for ink, capable of rapidly absorbing large amounts of ink, showing excellent color forming ability and capable of suppressing image deterioration caused by dye displacement that occurs when an image is stored in humid conditions and image deterioration caused by light when a printed image is displayed, and providing a printed image showing excellent long-term stability. The invention also provides a recording medium for ink having at least one layer provided on a substrate, and an ink receiving layer containing alumina hydrate as an outermost layer. A surface of the substrate at least on the side of the ink receiving layer is subjected to a cationizing treatment. An undercoat layer is provided on the same side as the cationizing treatment, to obtain cations in a predetermined distribution. The outermost ink receiving layer is provided on the undercoat layer.

**15 Claims, 2 Drawing Sheets**



**US 7,255,901 B2**

Page 2

## U.S. PATENT DOCUMENTS

|                  |         |                      |           |    |               |         |
|------------------|---------|----------------------|-----------|----|---------------|---------|
| 5,955,185 A      | 9/1999  | Yoshino et al. ....  | 428/304.4 | JP | 8-324100 A    | 12/1996 |
| 5,965,252 A      | 10/1999 | Santo et al. ....    | 428/329   | JP | 8-338000 A    | 12/1996 |
| 6,203,899 B1     | 3/2001  | Hirose et al. ....   | 428/341   | JP | 9-66663 A     | 3/1997  |
| 6,436,514 B1     | 8/2002  | Ishiyama et al. .... | 428/195   | JP | 9-66664 A     | 3/1997  |
| 6,511,736 B1     | 1/2003  | Asano et al. ....    | 428/195   | JP | 9-76628 A     | 3/1997  |
| 2001/0016249 A1  | 8/2001  | Kitamura et al. .... | 428/195   | JP | 11-105414 A   | 4/1999  |
| 2001/0055055 A1  | 12/2001 | Eguchi et al. ....   | 347/105   | JP | 11-291621 A   | 10/1999 |
| 2003/0152721 A1  | 8/2003  | Barcock et al. ....  | 428/32.35 | JP | 2000-198268 A | 7/2000  |
| 2004/0058098 A1* | 3/2004  | Kondo et al. ....    | 428/32.1  | JP | 2001-10220 A  | 1/2001  |
|                  |         |                      |           | JP | 2001-138628 A | 5/2001  |
|                  |         |                      |           | JP | 3204749 B2    | 9/2001  |

## FOREIGN PATENT DOCUMENTS

|    |              |        |    |               |         |
|----|--------------|--------|----|---------------|---------|
| EP | 1 080 938 A2 | 3/2001 | JP | 2001-341412 A | 12/2001 |
| EP | 1 226 959 A2 | 7/2002 | JP | 2002-225423 A | 8/2002  |
| JP | 57-44605 B2  | 9/1982 | JP | 2002-307823 A | 10/2002 |
| JP | 7-76161 A    | 3/1995 | JP | 2002-321445 A | 11/2002 |
| JP | 7-89220 A    | 4/1995 | JP | 2003-94800 A  | 4/2003  |
| JP | 7-232473 A   | 9/1995 | JP | 2003-165269 A | 6/2003  |
| JP | 8-132731 A   | 5/1996 | JP | 2003-191633 A | 7/2003  |
| JP | 8-230311 A   | 9/1996 |    |               |         |

\* cited by examiner

FIG. 1



**FIG. 2****FIG. 3****FIG. 4**

## 1

RECORDING MEDIUM FOR INK AND  
METHOD FOR PRODUCING THE SAME

This application is a continuation of International Application No. PCT/JP03/07000 filed on Jun. 3, 2003, which claims the benefit of Japanese Patent Application No. 162910/2002, filed Jun. 4, 2002.

## BACKGROUND OF THE INVENTION

## 1. Field of the Invention

The present invention relates to a recording medium for ink, particularly a recording medium for ink suitable for ink jet recording, and a method for producing a recording medium for ink. More specifically, the present invention relates to a novel recording medium which is improved with respect to the displacement of a coloring agent in the recording medium, generated in an image after the coloring agent contained in an ink is received as a fixed image, and a substrate (base paper) on which an ink receiving layer is to be formed. The present invention provides a recording medium for ink capable of suppressing image deterioration resulting from coloring agent (dye) displacement, which tends to be caused particularly during storage in a high humidity environment, or image deterioration caused by light when a printed image is displayed, thereby providing a printed image exhibiting excellent stability over time. The present invention also relates to a method for producing a recording medium for ink.

## 2. Related Background Art

Recently, as a recording medium for ink having a high ink absorbability and capable of providing a high quality image, there is being commercialized a recording medium for ink having an ink receiving layer which employs an alumina hydrate as an inorganic pigment. The recording medium for ink having the ink receiving layer employing such alumina hydrate, because of a positive charge of the alumina hydrate, shows a satisfactory fixation of the dye constituting the coloring agent in the ink and a satisfactory transparency, thereby providing advantages in comparison with the prior art recording media for ink such as a higher print density, an improved color development in the image, a higher surface glossiness and an image of photographic gradation.

Also, because of the increasing popularity of digital cameras, the recording medium for ink for recording the image information thereof is required to have a photograph-like glossy feeling in addition to a high image quality, in order to obtain an image close to a silver halide photograph. In the recording medium for ink having an ink receiving layer employing an alumina hydrate as mentioned above, if the substrate is a film, the ink receiving layer is formed by applying a coating liquid containing the alumina hydrate to obtain an image having a photographic glossiness. On the other hand, if the substrate is a fiber-based one, namely paper, the photographic glossiness cannot be obtained even by employing a coating liquid containing alumina hydrate for forming the ink receiving layer, and a super calendering or a cast coating is employed for providing the ink receiving layer with a gloss. In such case, a glossy image closer to the silver halide photograph can be obtained by a recording medium for ink processed by the cast process.

Such ink receiving layer containing alumina hydrate has a coloring agent fixing function because alumina functions as a cationic reactive material for an anionic dye, and, in order to further improve such function, Japanese Patent Application Laid-open Nos. 9-66663 (reference 1) and 2001-341412 (reference 2) disclose inventions for enhanc-

## 2

ing such function. Reference 1 describes application of a cationic treatment also on an outermost layer, and reference 2 describes application of a cationic treatment on the fibers of the substrate. Also, Japanese Patent Application Laid-open No. 8-230311 (reference 3) discloses a technology of causing a cationic surfactant to penetrate into an outermost layer.

On the other hand, to counteract the so-called rear penetration phenomenon caused by penetration of the recorded ink through the substrate and a re-displacement of the coloring agent, reaching the substrate, by deposition of water, Japanese Patent No. 3204749 (reference 4) discloses an invention of providing a layer containing a cationic polymer resin between the substrate and the ink receiving layer. According to this invention, after coating and drying of a coating liquid in which a water-soluble cationic polymer resin is dissolved in water, an ink receiving layer is formed with a coating liquid containing a pigment such as silica and a binder. This invention provides an intermediate layer containing a cationic polymer in order to intercept the coloring agent that can reach the substrate. Similarly, Japanese Patent Application Laid-open No. 11-105414 (reference 5) describes a recording medium having an undercoat layer between the substrate and the ink receiving layer, in which the undercoat layer contains at least one water-soluble cationic resin.

Also, the recording material for recording the aforementioned image information is being required to have a photograph-like glossiness in order to obtain an image close to a silver halide photograph. In order to meet such requirement, it is already known that a recording medium of a high glossiness can be obtained by employing a cast process on a recording medium having an ink receiving layer employing alumina hydrate and polyvinyl alcohol as binders. In particular, Japanese Patent Application Laid-open No. 2001-138628 (reference 6), for providing a high gloss medium for ink jet recording, discloses an invention of employing re-swelling as a technology for improving the cast process.

Formation of an ink receiving layer employing alumina hydrate and polyvinyl alcohol as binders is already known, but a viscosity increase with time in the coating liquid containing alumina hydrate and polyvinyl alcohol is an important factor. This is partly recognized in Japanese Patent Application Laid-open No. 7-76161 (reference 7). The reference 2 proposes, in order to solve the problem of fine cracks generated in drying the above-mentioned coating liquid, an alumina sol coating liquid containing alumina hydrate, polyvinyl alcohol and a predetermined amount of boric acid or a borate salt and a resinous film coated with such liquid (however, this reference only considers the coating liquid directly coated on the resinous film and only discloses coating of the liquid in one point where the ink receiving layer is 23 g/m<sup>2</sup>). On the other hand, Japanese Patent Application Laid-open No. 11-291621 (reference 8) cites the reference 2 and points out the difficulty of stable coating with the coating liquid disclosed in the reference 2 (references 7, 8 being by the same applicant). Reference 8 is based on a technical concept denying the improvement in the coating liquid and discloses a substrate paper which is obtained by sizing and drying a base paper principally formed by paper and prior to the coating process. More specifically, this invention prepares in advance a base paper by drying boric acid or the like of 0.5 to 1.5 g/m<sup>2</sup> and a paper surface treating agent (surface reinforcing agent or surface sizing agent) with a size pressing. In an example in reference 8, after the preparation of such base paper, a coating liquid constituted of boemite and polyvinyl alcohol and not con-

taining a crosslinking agent is prepared, and the prepared coating liquid is applied on the aforementioned base paper. The size pressing means, which is generally for improving water resistance, surface smoothness, printability etc. of the base paper, is used to slightly coat or impregnate the surface of the base paper with the sizing agent, which then is dried, for example, with a drum dryer. Therefore, the aforementioned references 7, 8 recognize the viscosity increase in the coating liquid, which is a drawback in the prior technology, but reference 7 merely tries to find a solution in the composition of the coating liquid, while reference 8 merely tries to find a solution in the base paper.

#### SUMMARY OF THE INVENTION

A cationic substance for an ink receiving layer, recognized in the prior technology, is mixed in a coating liquid (containing a pigment such as alumina hydrate and a binder) for forming the ink receiving layer, but cannot be mixed in an amount sufficient for fixing the coloring agent because it causes gelation of the coating liquid. In particular, alumina hydrate, if employed as a pigment, can be used only in a small amount as it causes an evident problem. On the other hand, if the cationic substance is provided or impregnated in an outermost layer of the ink receiving layer, the coloring agent is localized at the surface and thus increases the image density, but the coloring agent overflows in the lateral direction (hereinafter called lateral diffusion) instead of penetrating in the direction of the thickness of the recording medium, thereby deteriorating the sharpness of the image. Also, because of the localization of the coloring agent at the surface of the recording medium, light fastness and moisture resistance are not good. These tendencies become more conspicuous as the amount of the ink deposited on the recording medium increases. Also, under a high humidity environment, the fixed coloring agent, being soluble in water, may cause lateral diffusion in the recording medium, thereby causing a substantial deterioration of the image. Also, between adjacent images of different colors, the lateral diffusion forms another color, whereby the image may become different from the proper image.

A principal object of the present invention is to provide a recording medium capable of preventing the deterioration of the image caused by the aforementioned lateral diffusion, by taking the re-displacement or the fixing mechanism of the coloring agent into consideration to deal with the response of the cationic substance to the coloring agent, which has not been solved in the prior technology. It is also a principal object of the present invention to provide a production method capable of securely realizing such characteristics.

Another object of the present invention is to provide an invention capable of preventing the aforementioned lateral diffusion, by defining the construction of the substrate itself on which the ink receiving layer is to be formed. Still another object of the present invention is to provide a recording medium that more fully exploits the characteristics of the ink receiving layer, thereby preventing the rear penetration problem and forming and maintaining a sharp image. Another object of the present invention is to provide a recording medium for ink for ink jet recording, capable of rapidly absorbing a large amount of ink, having an excellent color developing property and is reliably producible and is capable of forming a high quality image with suppressed crack formation in the ink receiving layer, and a method for producing the recording medium for ink. Also, another object of the present invention is to provide a recording medium for ink for ink jet recording, capable of suppressing

image deterioration caused by dye displacement, which tends to appear particularly when an image is stored under a high humidity condition, and image deterioration caused by light when a printed image is displayed, and that provides a printed image showing excellent stability over time, and a method for producing the recording medium for ink.

As a result of intensive investigations for meeting the aforementioned objects, the present inventors have found that the cationic substance is desirably not mixed in the coating liquid constituting each layer such as the ink receiving layer but is diffused by penetration from a lower surface, that the ink receiving layer exhibit its characteristics preferably without addition of such cationic substance, and that the lateral diffusion phenomenon of the coloring agent in the ink takes place at an interface between the layers. More specifically, the cationic substance is made to gradually increase for the permeating liquid containing the coloring agent (preferably the cationic substance is made absent at the start of such increase thereby facilitating reception of the moving coloring agent at a lower side and, at the interface of two layers, the permeation toward the lower layer is accelerated so as to resist the lateral diffusion). Thus, the permeating liquid can be made to proceed relatively in the direction of the thickness of the recording medium without much lateral diffusion, even in the case where association or aggregation of the coloring agent takes place. As a result, it is rendered possible to secure the sharpness of the image and to significantly reduce bleeding of the image caused by lateral diffusion.

The present invention is based on this fact and provides, as a first invention, a recording medium for ink having an ink receiving portion for receiving an ink and holding a coloring agent of the ink, wherein an increasing region, in which a reactive substance capable of reacting with the coloring agent to hold the coloring agent is present with such a distribution as to increase in the direction of depth in the ink receiving portion, is provided in a position apart from the outermost ink recording surface of the recording medium for ink. According to this first invention, a cationic substance having the above-mentioned distribution is capable of suppressing image deterioration which results from displacement of the dye absorbed in the ink receiving layer and which tends to appear under a high humidity environment.

In addition to the first invention, it is preferred that the ink receiving portion includes an interface, which is a boundary of two different layers, that the above-mentioned increasing region does not include the interface of such two different layers, that a decreasing region, in which the reactive substance is present in such a distribution as to decrease in the direction of depth of the ink receiving portion, is provided in a position more distant from the side of the ink recording surface than the above-mentioned increasing region, that the ink receiving portion includes an alumina hydrate layer at the side of the above-mentioned ink depositing surface and the increasing region is not present in the alumina hydrate layer, that the ink receiving portion includes an alumina hydrate layer at the side of the ink depositing surface and the distribution of the maximum concentration in the increasing region is not present in the alumina hydrate layer, and that the ink receiving portion includes an interface, which is a boundary of two different layers, and the increasing region is formed starting from such interface not containing the reactive substance.

Also, the substrate of the present invention is a substrate, for a recording medium for ink, on which there is formed an ink receiving layer containing at least a pigment for holding the coloring agent of the ink and a binder for such pigment,

including an increasing region in which a reactive substance capable of reacting with the coloring agent thereby holding the coloring agent is present in such a distribution as to increase in the direction of depth as viewed from a surface on which the ink receiving layer is to be formed. Thus the aforementioned problems can be solved by the characteristics of the substrate, even excluding the formation of the ink receiving layer. Because of the aforementioned reasons, the substrate of the present invention preferably does not include the reactive substance on the surface on which the ink receiving layer is to be formed.

Still other features and effects relating to the relationship with the ink receiving layer of the present invention will be understood from the following description.

#### BRIEF DESCRIPTION OF THE DRAWINGS

FIG. 1 is a view showing a cross section of a recording medium for ink of the present invention and showing a relative distribution of a cation ( $N^+$ ) in corresponding positions;

FIG. 2 is a flow chart showing a producing method, not including a cast step, for a recording medium in an embodiment relating to the ink receiving layer;

FIG. 3 is a flow chart showing a producing method, including a cast step, for a recording medium in an embodiment relating to the ink receiving layer; and

FIG. 4 is a schematic view showing the configuration of a recording medium produced by the producing method for a recording medium in an embodiment relating to the ink receiving layer.

#### DETAILED DESCRIPTION OF THE PREFERRED EMBODIMENTS

In the following, the present invention will be clarified in detail by a preferred embodiment. The recording medium of this embodiment has the features that one or more layers are provided on a substrate, that an ink receiving layer containing alumina hydrate is provided on the outermost layer thereof, that a surface of the substrate on the side of the ink receiving layer is subjected to a cationizing treatment and that an undercoat layer laminated with the ink receiving layer has a distribution of the cation as in an increasing region A shown in FIG. 1.

FIG. 1 is a view showing a cross section of a recording medium for ink of the present invention and showing a relative distribution of a cation ( $N^+$ ) in corresponding positions, and indicates the relative proportion of cations obtained by measuring a magnified cross section of the recording medium of an embodiment 1 to be explained later. Numeral 1 indicates a paper-based substrate constituted of a base paper, and a water-soluble cation treated surface is formed on a surface thereof. Numeral 2 indicates an undercoat layer, formed by applying a coating liquid containing a pigment and a binder on the above-mentioned cation treated surface whereby cations diffuse from the lower surface. Numeral 3 indicates an ink receiving layer, formed by applying a coating liquid for the ink receiving layer on a surface, provided with anions, of the undercoat layer 2. In the ink receiving layer 3, cations of the aforementioned cationic treatment are not present as indicated by D (chart showing irregularities because of noise in measurement). On the other hand, the undercoat layer 2 includes a region A in which the cations gradually increase in the direction of thickness from the interface with the ink receiving layer 3 in which the cations of the aforementioned cationic treatment

are not present, a maximum portion B and a region C in which the cations gradually decrease from the maximum portion in the direction of thickness. "H" schematically indicates the range of the ink receiving portion of the present invention.

In the following there will be explained the substrate, the ink receiving layer and the undercoat layer constituting the recording medium for ink of the present invention, and producing methods therefor.

A preferred example of the substrate employed in the present invention can be a substrate capable of evaporating water or a solvent component from the rear surface of the substrate at the drying of the ink receiving layer, executed in a cast step for forming a glossy surface on the recording medium for ink, and there is particularly preferred a fibrous substrate, namely paper. As such paper, there can be employed a base paper prepared by employing pulp, which can be wood pulp, for example, chemical pulp such as LBKP or NBKP, mechanical pulp such as GP, PGW, RMP, TMP, CTMP, CMP or CGP, used paper pulp such as DIP, or non-wood pulp such as kenaf, bagasse or cotton and an already known pigment as main components and mixing at least one of the various additives such as a binder, a sizing agent, a fixing agent, a yield improving agent, a cationizing agent, or a paper strength increasing agent. The base paper is produced with various apparatus such as a Fourdrinier paper machine, a cylinder paper machine or a twin wire paper machine. Alternatively, a base paper may be prepared by forming, on the aforementioned base paper, with a size press or an anchor coat layer with starch, polyvinyl alcohol etc., or a coated paper such as art paper, coated paper or cast coat paper prepared by forming a coated layer on such base paper.

The recording medium for ink of the present invention is 35 featured in that at least a side of the ink receiving layer of the substrate such as the base paper or the coated paper mentioned above is subjected to a cationizing treatment. Therefore, in producing the recording medium for ink of the present invention, it is necessary to execute the cationizing 40 treatment on the substrate prior to the formation of the undercoat layer to be laminated with the ink receiving layer. The cationizing treatment is preferably executed with a processing liquid containing at least one of the cationic substances listed in the following. Prior to the cationizing 45 treatment of the substrate, if necessary, the substrate may be subjected to size adjustment with a sizing agent, or there may be provided another layer such as an adhesion promoting layer. Also, there may be executed a corona treatment in order to improve the adhesion between the cationizing substance for cationizing the substrate and the substrate.

The cationic substance to be employed in the present invention is not particularly limited as long as it includes a molecule with a cationic portion. For example, there can be employed a cationic surfactant of the quaternary ammonium 55 salt type such as monoalkylammonium chloride, dialkylammonium chloride, tetramethylammonium chloride, trimethylphenylammonium chloride, or ethylene-oxide-added ammonium chloride, or a cationic surfactant of the amine salt type, or an amphoteric surfactant such as alkylbetain, imidazolium betain or alanine which includes a cationic portion.

There can also be employed a polymer or an oligomer having a cationic property. Examples of the polymer or the oligomer having cationic property include a cation-modified product of polyacrylamide, a copolymer of acrylamide and a cationic monomer, polyethylenimine, a polyamide-epichlorhydrin resin, polyaminepolyamide epichlorhydrin,

polyvinylpyridinium halide, a dimethyldiallylammonium chloride polymer, polyamidamine, polyepoxyamine, dicyanodiimide-formalin condensate, or various polyamine resins such as polyallylamine, polyaminesulfon, or polyvinylamine. There can also be employed a homopolymer of a vinylpyrrolidone monomer or a copolymer thereof with another ordinary monomer, a homopolymer of vinyloxazolidone monomer or a copolymer thereof with another ordinary monomer, a homopolymer of vinylimidazole monomer or a copolymer thereof with another ordinary monomer. The ordinary monomer mentioned above can be, for example, methacrylate, acrylate, acrylonitrile, vinylether, vinyl acetate, ethylene or styrene.

Among these cationic substances, there is particularly preferred an alkyl (meth)acrylate quaternary ammonium salt having a benzyl group, or a cationic resin such as a polymer or a copolymer including an alkyl (meth)acrylamide quaternary ammonium salt as a skeleton. In case of employing an anion (borate ion) for forming a salt with a metal ion as in the following example, such cationic polymer or cationic organic substance is preferred for obtaining the aforementioned cation distribution.

Although not particularly restricted, an amount of the cationic substance employed in the cationizing treatment is preferably 0.1 to 5 g/m<sup>2</sup> in terms of solid, more preferably 0.5 to 3 g/m<sup>2</sup>. In a preferred embodiment of the recording medium for ink of the present invention, a glossy surface is provided on at least one surface thereof in order to enable formation of an image of photographic quality, and, in such case, an amount of the cationic substance, employed for the cationizing treatment of the substrate, exceeding 5 g/m<sup>2</sup> may deteriorate the surface property or the glossiness of the glossy surface. More specifically, the formation of a glossy surface is executed, for example, by drying a material forming the ink receiving layer and constituting the outermost layer of the recording medium for ink in contact, while in a wet state, with a heated mirror surface. In such operation, a large amount of the cationic substance employed for the cationizing treatment provides a thick and dense treated layer, whereby the surface property or the glossiness of the glossy surface of the recording medium for ink may be deteriorated. Also, an amount exceeding 3 g/m<sup>2</sup> shows a slight loss of the surface property and the glossiness in comparison with a case of 0.5 to 3 g/m<sup>2</sup>.

The cationizing treatment of the surface of the substrate can be achieved by an already known method, for example by coating with a coating apparatus such as a roll coater, a blade coater, a gate roll coater, a bar coater, a size press, a curtain coater, an air knife coater, a spray coater or a (micro)gravure coater. In the cationizing treatment of the substrate of the present invention, it is particularly preferred to employ a blade coater, a size press or a (micro)gravure coater in consideration of the coating productivity.

The cationizing treatment of the surface of the substrate is completed by drying thereafter with a hot air oven, or a heated drum. Also if necessary, in order to improve the smoothness or the surface strength of the cationized surface of the substrate, a calendering or super calendering process may be applied.

The recording medium for ink of the present invention is formed by applying a cationizing treatment on the surface of the substrate as explained in the foregoing, and forming, on such substrate, at least an undercoat layer and an outermost ink receiving layer laminated thereon. In the following, the undercoat layer will be explained.

The substrate, which is composed of a base paper or a coated paper as explained in the foregoing and the surface of

which is subjected to the cationizing treatment, may be directly provided with an undercoat layer, but there may also be applied a calendering process for surface smoothing or thickness adjustment of the substrate. Also, in consideration of evaporation of water or solvent component from the rear surface of the substrate and of ease of coating of the undercoat layer, it is preferred to employ a substrate having an air permeability of 20 to 500 seconds determined by JISP8117. In case the air permeability of the substrate is less than the above-mentioned range, namely in case of a substrate of a lower density, printing on a recording medium for ink utilizing such substrate may result in swelling of the substrate due to ink absorption, thereby causing waviness and the inability to obtain a quality comparable to that of a silver halide photograph. On the other hand, in a substrate with the air permeability exceeding the above-mentioned range, a satisfactorily glossy surface may not be obtained because the water or solvent component cannot easily evaporate from the rear surface of the substrate at the casting process.

In consideration of the above-mentioned reasons for prevention of loss of the gloss obtained by the cast process, it is advantageous to employ, in the present invention, a substrate having a Stöckigt sizing degree (JISP8122) within a range of 20 to 300 seconds and a Bekk smoothness (JISP8119) within a range of 10 to 60 seconds. Also in order to obtain a recording medium comparable in quality to a silver halide photograph and having stiffness at an A4 size or larger, it is preferred to employ a substrate of a basis weight of 140 to 200 g/m<sup>2</sup> and a Gurley stiffness (JISP8125, machine direction) of 3 to 15 mN. In producing the recording medium for ink of the present invention, it is preferred to employ a substrate of which the basis weight, thickness, ash content, internal size amount and surface size amount are suitably selected and adjusted so that the characteristics of the substrate remain within the above-mentioned ranges.

The recording medium for ink of the present invention, in which at least a substrate surface on the side of the ink receiving layer is subjected to a cationizing treatment and which includes at least an undercoat layer and an outermost ink receiving layer laminated on such undercoat layer, on the side of the ink receiving layer, is capable of rapidly absorbing a large amount of ink, shows an excellent color forming ability and is capable of forming a high quality image with suppressed crack formation in the ink receiving layer. Particularly, it can suppress generation of image deterioration due to dye displacement, which may take place if the image is maintained under a high humidity environment, and generation of an image deterioration by light if the image is displayed, thereby providing excellent stability over time of the printed image.

According to the investigations of the present inventors, among the aforementioned effects, the effects against the generation of image deterioration under the high humidity environment and against the generation of image deterioration by light can be particularly securely obtained by forming an undercoat layer between the ink receiving layer and the substrate subjected to the cationizing treatment. In the recording medium for ink of the aforementioned construction, the cationic substance present under the undercoat layer suppresses the generation of image deterioration resulting from displacement of the dye absorbed in the ink receiving layer.

At the time when the cationizing treatment of the surface of the substrate 1 and lamination of the undercoat layer 2 thereon are carried out, the cationic substance is localized in the vicinity of the surface of the substrate 1 and is scarcely

present on the outermost surface of the undercoat layer 2. In such case, the cationic substance employed in the cationizing treatment can be thereafter diffused in the undercoat layer to form the aforementioned distribution of the cationic substance, in the course of coating and drying of the undercoat layer, coating and drying of the outermost ink receiving layer, or formation of the glossy surface by drying the outermost ink receiving layer in a wet state or a re-wetted state in contact with the heated mirror surface. In this manner it is rendered possible to effectively suppress the dye displacement in the ink receiving layer, which tends to appear in a high humidity environment, and the image deterioration resulting therefrom.

On the other hand, in order to suppress the image deterioration resulting from dye displacement in the ink receiving layer under a high humidity environment, it is also conceivable to mix the cationic substance in a coating liquid for forming the outermost ink receiving layer, but the investigation of the present inventors indicates that the amount of addition to alumina hydrate is quite limited and cannot effectively suppress the image deterioration resulting from dye displacement under a high humidity environment. Also, depending upon the amount of addition, the coating liquid may gel or coagulate in the course of preparation thereof, whereby the formation of the ink receiving layer becomes impossible. Also, though the formation of the ink receiving layer is possible if the coating liquid does not gel or coagulate, but the effect for suppressing image deterioration due to light when the image is displayed becomes evidently inferior to that in the construction of the present invention. The present inventors hypothesize that this is because the cationic substance is selectively present to a great extent in the ink receiving layer constituting the outermost surface of the recording medium for ink in the above-described case, in contrast to the aforementioned distribution of the cationic substance. It is also conceivable, in order to obtain an effect similar to that of the present invention, to mix the cationic substance in a coating liquid for forming the undercoat layer. However, in such case, like the above-mentioned case, the alumina hydrate and the cationic substrate show a very high possibility of gelation or aggregation, whereby, depending on the amount of the cationic substance contained in the undercoat layer, crack formation in the outermost ink receiving layer or loss in the surface gloss may be caused.

In the following, there will be explained material for forming the undercoat layer constituting the recording medium for ink of the present invention. The undercoat layer can be formed by a coating liquid including a pigment and a binder, but is preferably provided with an ink receiving property. For the pigment, there can be employed at least one selected from inorganic pigments such as light calcium carbonate, heavy calcium carbonate, magnesium carbonate, kaolin, talc, calcium sulfate, barium sulfate, titanium dioxide, zinc oxide, zinc sulfide, zinc carbonate, satin white, aluminum silicate, diatomaceous earth, calcium silicate, magnesium silicate, synthetic amorphous silica, colloidal silica, alumina, alumina hydrate, aluminum hydroxide, lithopone, zeolite, and hydrogenated halocite, and organic pigments such as styrenic plastic pigments, acrylic plastic pigments, polyethylene particles, microcapsule particles, urea resin particles and melamine resin particles.

For the binder, there can be employed, without any particular restriction, any material capable of forming a film by binding the above-mentioned pigment and not hindering the effects of the present invention. For example, there can be employed a starch derivative such as oxidized starch,

etherized starch, or phosphate esterized starch; a cellulose derivative such as carboxymethyl cellulose, or hydroxyethyl cellulose; casein, gelatin, soybean protein, polyvinyl alcohol or a derivative thereof; a conjugate polymer latex such as polyvinylpyrrolidone, a maleic anhydride resin, a styrene-butadiene copolymer, or a methyl methacrylate-butadiene copolymer; an acrylic polymer latex such as of a polymer or a copolymer of an acrylate ester or a methacrylate ester; a vinylic polymer latex such as an ethylene-vinyl acetate copolymer; a functional group-modified polymer latex, for example, of the foregoing polymers modified with a monomer containing a functional group such as a carboxyl group; foregoing polymers which are rendered cationic with a cationic group, rendered cationic at their surfaces with a cationic surfactant, polymerized in the presence of a cationic polyvinyl alcohol to obtain a distribution of such polyvinyl alcohol on the polymer surface, or polymerized in a suspension liquid of cationic colloid particles to obtain a distribution of such particles on the polymer surface; an aqueous binder of a thermosettable resin such as melamine resin or urea resin; a polymer or copolymer synthetic resin of an acrylate ester or a methacrylate ester such as polymethyl methacrylate; or a synthetic resin binder such as polyurethane resin, unsaturated polyester resin, vinyl chloride-vinyl acetate copolymer, polyvinylbutyral, or alkyd resin. These binders may be used singly or in a combination of two or more kinds.

The undercoat layer can be easily formed by applying and drying a coating liquid, containing the pigment and the binder as explained above, on the surface of the substrate. The undercoat layer is formed at least on a surface of the substrate on the side of the ink receiving layer, but it is also possible to form the undercoat layer on the rear surface, thereby providing the undercoat layers on both sides of the substrate. In consideration of stability of environmental curling of the recording medium for ink, the undercoat layer is preferably formed on both sides of the substrate. In order to sufficiently cover surface fibers, such as cellulose pulp constituting the substrate, the undercoat layer preferably has a dry coating amount of 10 g/m<sup>2</sup> or higher, more preferably 15 g/m<sup>2</sup> or higher. A dry coating amount less than 10 g/m<sup>2</sup> is insufficient for completely covering the surface fibers such as cellulose pulp of the substrate, whereby the glossiness may be affected.

Also, the amount of the binder in the coating liquid for forming the undercoat layer is preferably 5 to 50 mass % with respect to the pigment. A binder amount less than the above-mentioned range tends to generate cracks in the undercoat layer and to result in an insufficient mechanical strength of the undercoat layer, thereby causing powder falling. Also, an amount exceeding the above-mentioned range tends to deteriorate the absorbability for the solvent of the ink and the evaporation of water etc. (vapor movement to the rear surface of the substrate) in the casting process. In the present invention, a calendering process may be executed if necessary after the formation of the undercoat layer, thereby making it possible to adjust the thickness of the substrate/undercoat layer.

In consideration of evaporation of water or the solvent component from the rear surface of the substrate, also of the coating property (wetting property) in first and second surface treatment steps to be explained later, and of the coating property for the outermost ink receiving layer to be formed thereafter, it is preferred, for the recording medium for ink of the present invention, that the substrate having the undercoat layer on both sides has an air permeability of 1,500 to 5,000 seconds (JISP8117). It is also desirable for it

## 11

to have a Stöckigt sizing degree of 100 to 400 seconds and a Bekk smoothness of 100 to 500 seconds. These characteristics can be obtained by suitably controlling the composition and the dry coating amount of the undercoat layer, and the presence or absence of a calendering process. Also, in order to obtain a recording medium comparable in quality to a silver halide photograph and having stiffness at an A4 size or larger, it is preferred to adjust the substrate and the undercoat layer so as to have a basis weight of 160 to 230 g/m<sup>2</sup> and a Gurley stiffness (JIS P8125, machine direction) of 7 to 15 mN.

In the following, there will be explained a method of forming the ink receiving layer laminated on the undercoat layer explained above. In such case, it is preferred to prepare the recording medium for ink by applying, to the undercoat layer, a surface treatment constituted of two steps explained in the following, and then forming the ink receiving layer. The surface treatment to be executed in such case is preferably constituted by a first surface treatment step of applying a coating liquid containing one or more compounds selected from the group of boric acid and borate salts on the undercoat layer and drying such undercoat layer, and a second surface treatment step of applying, on the undercoat layer after the first surface treatment step, a coating liquid containing one or more compounds selected from the group of boric acid and borate salts. It is further preferred that the ink receiving layer is formed while the coating liquid coated in the second surface treatment step is still in a wet state.

The coating liquid, containing one of more compounds selected from the group of boric acid and borate salts and to be employed in the surface treatment of the undercoat layer, most preferably contains borax (sodium tetraborate) in consideration of the ability for suppressing crack formation.

For preparing the recording medium for ink of the present invention, the outermost ink receiving layer is formed after the aforementioned surface treatment is applied to the undercoat layer. In the following, there will be given an explanation of the ink receiving layer of the present invention. The ink receiving layer can be formed in general by applying a coating liquid including a pigment as explained below, and a binder. There can be employed an inorganic pigment such as a light calcium carbonate, heavy calcium carbonate, magnesium carbonate, kaolin, aluminum silicate, diatomaceous earth, calcium silicate, magnesium silicate, synthetic amorphous silica, colloidal silica, alumina, alumina hydrate or magnesium hydroxide; or an organic pigment such as styrenic plastic pigments, acrylic plastic pigments, polyethylene particles, microcapsule particles, urea resin particles or melamine resin particles. In the recording medium for ink of the present invention, as a main component of the ink receiving layer, there is employed alumina hydrate which is particularly preferred in the dye fixability, transparency, print density, color forming property and glossiness, among the foregoing substances. In the coating liquid for forming the ink receiving layer, the content of alumina hydrate is preferably from 60 to 100 mass % with respect to the inorganic pigment contained in the coating liquid.

The present invention also provides a further preferred embodiment in the relation between the formed state of the ink receiving layer and the aforementioned cation distribution. The aforementioned cation distribution can be formed by diffusing a water-soluble cationic resin not in the ink receiving layer but in the undercoating layer lying thereunder from a lower surface thereof into the interior thereof, and by diffusing an anionic substance from an upper surface thereof constituting an interface with the ink receiving layer. Thus, a distribution is obtained in which the cationic sub-

## 12

stance gradually increases in the direction of depth (cf. FIG. 1). In the following there will be explained a preferred embodiment in which the anionic substance is also used as a crosslinking agent for the binder. The mechanism of formation of the ink receiving layer has been investigated from various view points, in order to achieve fundamental technical analyses of the pigment and the binder contained in the coating liquid and the solvent employed for dissolving the binder. As a result, the present inventors have determined that it is important to generate a mechanism in which the binder, behaving as a dispersant for the pigment in the coating liquid, is positioned around the pigment, which starts to aggregate at the drying of the coating liquid, thereby binding such pigment in the coating liquid as long as possible. The inventors have also determined that it is important to obtain a uniform distribution of the binder in the ink receiving layer, since, as in the recording medium itself, a fluctuation in the distribution of the binder may form an area of lowered density due to excessive ink absorption or an area of reduced ink absorbability, thus causing deterioration of the image quality due to ink overflowing.

Technical aspects for meeting these criteria include a first goal of preventing the transfer of the binder together with the solvent in a large amount from the coating liquid to a surface to be coated (member to be coated), with the coating liquid, and securely crosslinking the binder in the vicinity of the interface between the coated surface and the coating liquid, then a second goal of utilizing the characteristics of the pigment, not only in forming the crosslinked state of the binder but also in causing an aggregation or a viscosity increase of the pigment and forming a rational pore distribution, also a third goal of providing a preferred form for forming the surface to be coated and a fourth goal of obtaining a recording medium prepared by a production method that achieves these goals and improving the recording characteristics obtained by the configurational features of the recording medium. More specifically, the present invention also has a technical goal that polyvinyl alcohol soluble in water (preferably purified water for preventing impurity to alumina) functions principally as a solute in water of the coating liquid for forming the ink receiving layer but does not diffuse together with water in the coated layer and performs a rapid functional change from the solute to a binder.

An embodiment relating to the ink receiving layer is based on a correlation between the structure of the ink receiving layer on the ink recording surface side thereof and the interior thereof, and a layer region including a surface to be coated on which the ink receiving layer is formed. This prevents the loss of the binder of the coating liquid into the side of the surface to be coated, utilizing a reaction rate or a reaction state at a liquid-liquid interface to achieve effective removal of the solvent present in the coating liquid, thereby attaining at least one of the aforementioned goals. In the embodiment relating to the ink receiving layer, there is used a term "layer region" involving a thickness, but a layer need not be formed in a complete form or may be formed as an area with a certain thickness.

In the aforementioned embodiment relating to the ink receiving layer, since it is preferred, at the aforementioned crosslinking reaction, to exclude the liquid component such as the solvent (water in case of PVA (preferably purified water in order to avoid impurity for alumina)) for dissolving the binder of the coating liquid, the recording medium preferably includes, as the substrate for supporting the ink receiving layer, a porous member (paper, pulp, porous layer

## 13

etc.) into which the liquid component of the coating liquid can permeate. In addition, in order to improve the adhesion and the strength of the ink receiving layer to the substrate (anchoring effect), it is also preferred that the aforementioned wet surface is not a smooth surface but has recesses for the coating liquid and that crosslinking of the binder occurs in such recesses. Further features of the embodiment relating to the ink receiving layer will be understood from the following description.

In the following, the embodiment relating to the ink receiving layer will be clarified further by a preferred embodiment. A preferred production method for the recording medium in the embodiment relating to the ink receiving layer is roughly classified into two forms shown in FIGS. 2 and 3. FIG. 2 shows a production method including two surface treating steps and a step of forming the ink receiving layer. FIG. 3 shows a production method for the recording medium, further including a cast step for providing surface gloss.

Now there will be explained a preferred form of the production method for the recording medium, in the embodiment relating to the ink receiving layer. The production method of the embodiment relating to the ink receiving layer is capable of obtaining an appropriate aggregating function of the pigment and a binding function of the binder securely at the liquid-liquid interface while maintaining the state of the coating liquid at the liquid-liquid interface, and also of preventing the loss of the binder which should be present in the ink receiving layer, thereby stabilizing the characteristics and providing a satisfactory productivity. The recording medium of the embodiment relating to the ink receiving layer has a novel construction that is realized as a result of retention of the binder to be present in the ink receiving layer, wherein the ink receiving layer includes a first layer region in which the binder is made relatively uniform with the pigment, and a second layer region in which the binder is crosslinked by a second crosslinking agent so as to reach a larger crosslinking degree than in the first layer region, and the first layer region is positioned closer, than the second layer region, to the ink recording surface.

In the embodiment relating to the ink receiving layer, at the formation of the ink receiving layer and in the final construction, the binder constituting the ink receiving layer can be positioned appropriately with respect to the pigment, so that a uniform pore distribution can be obtained by the pigment and the binder provided by the coating liquid. At the same time, a substantial barrier layer region capable of preventing the loss of the binder from the coating liquid is formed by a reaction state of a high speed and a high probability at the liquid-liquid interface, so that the crosslinking degree itself can be made larger. In order to achieve effective removal of the solvent in the coating liquid, since it is preferred, at the aforementioned crosslinking reaction, to exclude the liquid component such as the solvent (water in case of PVA (preferably purified water in order to avoid impurity for alumina)) for dissolving the binder of the coating liquid, the recording medium preferably includes, as the substrate for supporting the ink receiving layer, a porous member (paper, pulp, porous layer etc.) into which the liquid component of the coating liquid can permeate.

The embodiment relating to the ink receiving layer causes the binder, behaving as a dispersant for the pigment in the coating liquid, to be positioned around the pigment which starts to aggregate after the coating thereby binding such pigment, while maintaining the mixing proportion of the

## 14

pigment and the binder prior to the coating as long as possible, and utilizes the liquid-liquid interface mentioned above. It is thus possible to solve the problem in the ink receiving layer of a partial density loss resulting from excessive ink absorption and a partial image quality loss resulting from insufficient ink absorption, caused by the fluctuation of the binder, as may occur in the prior technology. In the embodiment relating to the ink receiving layer, it is possible to prevent the transfer of the binder together with the solvent in a large amount from the coating liquid to a surface to be coated (member to be coated) with the coating liquid and to securely crosslink the binder in the vicinity of the interface between the surface to be coated and the coating liquid. Also by utilizing the viscosity increasing property and the aggregating property (pH dependency in case of alumina hydrate) of the pigment, it is rendered possible not only to form a crosslinked state of the binder but also to obtain an aggregation or a viscosity increase of the pigment and to form a reasonable pore distribution. Moreover, the surface treatment in stepwise manner as explained in the following provides a uniform and stable surface to be coated. More specifically, in the embodiment relating to the ink receiving layer, polyvinyl alcohol soluble in water (preferably purified water for preventing impurity to alumina) functions principally as a solute in water in the coating liquid for forming the ink receiving layer but does not diffuse together with water in the coated layer and performs a rapid functional change from the solute to a binder. Also, the embodiment relating to the ink receiving layer can provide a recording medium which can rapidly absorb a large amount of ink, as required in a photoprinter recording, also can be produced in a stable manner even with an ink receiving layer of 30 g/m<sup>2</sup> or larger (amount after drying), can achieve a substantial control of the binder which functions also as a dispersant, and is excellent in ink absorbing property and color forming property, and also provides a production method, having satisfactory productivity, for the recording medium.

In a production method of the embodiment relating to the ink receiving layer, the substrate is subjected to a first surface treatment and a second surface treatment stepwise. A coating liquid to be employed in the first surface treatment step preferably provides a dry coating amount of 0.05 to 2.0 g/m<sup>2</sup> in terms of solid borax. An amount less than the aforementioned range results in an excessively low viscosity of the coating liquid, thereby leading to a frequent liquid flow, while an amount exceeding the aforementioned range tends to generate spot-shaped defects on the surface (cast surface) in the cast process, whereby a uniform and satisfactory glossy surface may not be obtained. In the first surface treatment step, a coating liquid containing at least one selected from the group of boric acid and borate salts, for example a 5% aqueous solution of borax, is applied on the undercoat layer, then dried and solidified. The coating liquid may further include a solvent such as alcohol for defoaming if necessary. The first surface treatment step, since a lower dry coating amount is preferred, can be executed at a considerably high coating and drying speed, for example as high as 50 to 200 meters per minute.

In a second surface treatment step, executed in succession to the first surface treatment step, a coating liquid containing at least one selected from a group of boric acid and borate salts, as in the first surface treatment step, is applied on the surface treated substrate already subjected to the first surface treatment step. In the second surface treatment step, different from the first surface treatment step, the coating liquid is not dried and solidified after the coating. More specifically, the

substrate surface is formed into a moist state of a certain level (which may be a liquid state or a viscosity increased state), and a next coating liquid for forming the ink receiving layer is applied while such state is maintained. In this operation, there is secured a reaction state by the liquid-liquid interface in the embodiment relating to the ink receiving layer. At this interface, the coating liquid for the ink receiving layer shows a faster gelling speed or a faster crosslinking speed. On the other hand, in case a reaction at the liquid-liquid interface cannot be obtained, the binder diffuses into the substrate or in the pores on the solidified surface formed by the first surface treatment, whereby an amount or a position of the binder for binding the pigment may be changed.

The aforementioned stepwise surface treatments provide the following advantage. In the first surface treatment step applied to the substrate, since the coating liquid is dried, boric acid or borate salt (hereinafter collectively called "borate salt etc.") is present as a solid on the substrate or in the undercoat layer (an upper part in the layer). Then, when the second surface treatment and the formation of the ink receiving layer are executed in this state, an aqueous solution of boric acid or a borate salt (hereinafter collectively called "borate processing solution etc.") coated in the second surface treatment step principally provides an advantage that a liquid surface can be secured by the borate processing solution etc. It is therefore also ensured that the coating liquid for forming the ink receiving layer in the next step and the borate processing solution etc. are contacted and mixed in a liquid-liquid state.

On the other hand, in case the coating liquid for forming the ink receiving layer and the borate salt etc. in solid state are contacted, the borate salt etc. in solid state dissolve in the coating liquid for forming the ink receiving layer over a certain time, during which the binder permeates from the liquid into the substrate, thereby generating a quantitatively deficient area. At the same time, the coating liquid in a portion where the borate salt etc. are dissolved reaches a concentration considerably higher than in a surrounding area, thereby causing a rapid local gelation or crosslinking and a local viscosity increase of the coating liquid to generate a "coating unevenness" in the interior and on the surface. Thus, the ink receiving layer becomes extremely non-homogeneous, including both an unnecessary giant pigment aggregation (resulting from deficiency of binder) and a bound state with the binder.

The use of the surface treatments in two steps allows formation of a moist state more stably with the borate processing solution etc., on the substrate on which the borate salt etc. are present in solid state. A rapid crosslinking reaction can be realized in a liquid-liquid contact interface on the undercoat layer of the above-mentioned state, while the solvent such as water in the coating liquid for forming the ink receiving layer can be separated from the binder and eliminated by the pores of the formed porous substance, whereby an ideal aggregation of the pigment and an appropriate binding by the binder can be formed in a homogeneous state. As a result, it is rendered possible to suppress crack generation resulting from a binder deficiency at the manufacture, and to form a thick ink receiving layer with a high dry coating amount.

Boric acid or borate salt to be employed in the second surface treatment step can be similar to that employed in the formation of the ink receiving layer or in the first surface treatment step, but it is preferred to employ borax in consideration of the gelling or crosslinking rate in the aforementioned step of forming the ink receiving layer, the

change in viscosity of the coating liquid for forming the ink receiving layer during the use thereof, and suppression of crack generation in the formed ink receiving layer. In the second surface treatment step, it is preferred to employ a coating amount such that the coating liquid does not overflow from the substrate after the first surface treatment. Though dependent on the absorbability of the substrate after the first surface treatment, it is preferred to make an adjustment since an overflowing state of the coating liquid for the second surface treatment may cause a floating state of the coating liquid for the ink receiving layer at the coating thereof, thereby deteriorating the adhesion of the ink receiving layer to the substrate.

It is also preferred, in the second surface treatment step, to adjust the solid concentration of one or more substances selected from the group of boric acid and borate salts so as to obtain a dry coating amount of 0.05 to 2.0 g/m<sup>2</sup> in terms of borax solid. In the second surface treatment step, a coating liquid containing one or more compounds selected from the group of boric acid and borate salts, for example a 5% aqueous solution of borax, is applied on the undercoat layer already subjected to the first surface treatment. The coating liquid may further include a solvent such as alcohol for defoaming if necessary.

Dry coating amounts of the coating liquids applied in the first and second surface treatment steps can be suitably determined from the relationship of the first surface treatment step and the second surface treatment step. For example, if the coating amount of the first surface treatment step is reduced, a compensation can be made by increasing the coating amount in the second surface treatment step. However, it is preferred to select the dry coating amount in the first surface treatment step from 0.1 to 1.0 g/m<sup>2</sup> in consideration of the ease of control on the coating amount and the relation with the coating amount in the succeeding second surface treatment step, and to select the dry coating amount in the second surface treatment step from 0.3 to 1.5 g/m<sup>2</sup> in consideration of the coating speed and the relation with the coating amount in the first surface treatment step.

The aforementioned moist surface is not a uniform surface but is made to have recesses for the coating liquid, and the crosslinking of the binder is caused in such recesses to secure the adhesion and the anchoring effect for the ink receiving layer to the substrate. Such construction having the crosslinked binder in the recesses is effective also for the formed recording medium. In the preparation of the coating liquid for the ink receiving layer, there is preferably employed a mixing apparatus which mixes one or more compounds selected from the group of boric acid and borate salts with an alumina hydrate dispersion, and mixes the thus-obtained mixture liquid with an aqueous solution of polyvinyl alcohol constituting the binder immediately prior to the coating, thereby obtaining a coating liquid. In this manner, it is possible to reduce the viscosity increase with time or the gelation appearing in the course of the manufacturing process, thereby improving the production efficiency. In the above-mentioned alumina hydrate dispersion, the pigment preferably has a solid concentration of 10 to 30 mass %. A concentration exceeding such range increases the viscosity of the pigment dispersion and that of the ink receiving layer, whereby difficulty may arise in the coating property.

In the undercoat layer to be explained later and in the aforementioned ink receiving layer, there may be suitably contained, if necessary, various additives such as a pigment dispersant, a viscosifier, a fluidity improving agent, a defoamer, an antifoamer, a releasing agent, a permeation

agent, a coloring pigment, a coloring dye, a fluorescent whitening agent, an ultraviolet absorber, an antioxidant, an antiseptic, an antimold agent, a water resistant agent, a dye fixing agent etc.

The formation of the ink receiving layer in the recording medium is presumed to be based on the following phenomena. It is firstly presumed that a reaction of boric acid or borate salt, employed in the surface treatment of the substrate, with polyvinyl alcohol in the coating liquid for the ink receiving layer, namely a gelation and/or a crosslinking reaction, (1) suppresses the permeation of polyvinyl alcohol into the undercoat layer, whereby the binder can be distributed relatively uniformly in the ink receiving layer, and, in a drying step in the formation of the ink receiving layer, (2) a movement of the coating liquid can be reduced by a viscosity increase owing to the gelation and/or the crosslinking reaction. Particularly, if alumina hydrate is used for forming the ink receiving layer, it is presumed that a crosslinking reaction of alumina hydrate and boric acid or borate salt generates so-called inorganic polymers, and the interaction of boric acid or borate salt, alumina hydrate and polyvinyl alcohol functions effectively for suppressing crack formation in the ink receiving layer.

The substrate to be employed in the embodiment relating to the ink receiving layer is not particularly restricted as long as it accepts a surface treatment to be explained later, but when forming a glossy surface by applying a cast step to the surface of the recording medium, there is preferred a fibrous substrate, namely a paper substrate, because water or a solvent component evaporates from the rear surface of the substrate. The paper substrate includes a base paper subjected to a sizing with starch, polyvinyl alcohol etc., and a coated paper such as art paper, coated paper or cast coated paper prepared by forming a coated layer on such base paper.

When forming a glossy surface by applying a cast step to the surface of the recording medium, it is preferred that the paper substrate is provided thereon with a coated layer of such a thickness as to completely cover the cellulose pulp fibers and the texture of the paper substrate (base paper), as an undercoat layer for the ink receiving layer. If such covering is not attained, there may easily arise a coating unevenness (streak defect etc.) derived from such fibers or texture, and the cellulose pulp fibers are present in the ink receiving layer, on the surface thereof or in the vicinity of such surface whereby, even when applying the cast process to the surface of the recording medium, it is difficult to obtain a satisfactorily uniform cast surface, namely, a photograph-like highly glossy surface. In order to cover the cellulose pulp of the paper substrate, the coated layer preferably has a dry coating amount of 10 g/m<sup>2</sup> or higher, more preferably 15 g/m<sup>2</sup> or higher. A dry coating amount of less than 10 g/m<sup>2</sup> is insufficient for completely covering the cellulose pulp or the texture of the substrate, whereby the glossiness may be affected.

The undercoat layer can be formed with a coating liquid containing the pigment and the binder, but preferably has an ink receiving property. The undercoat layer can be formed in one or more layers at least on a surface of the substrate. In consideration of stability of environmental curling of the recording medium, the undercoat layer is preferably formed on both sides of the substrate. The substrate to be employed in the embodiment relating to the ink receiving layer includes a paper substrate provided with the aforementioned undercoat layer. Also, in consideration of the evaporation of water or solvent component from the rear surface of the substrate in the cast step, the coating property (wetting

property) of the coating liquids to be applied on the substrate in the first and second surface treatment steps to be explained later, and the coating property of the material for forming the ink receiving layer on the substrate, the substrate preferably has a permeability (JIS P 8117) of 1,500 to 5,000 seconds. If the permeability is less than the above-mentioned range, the substrate has a low density, so that the crosslinking agent (boric acid or borate salt) in the first and second surface treatment steps shows a high penetration and 10 may not function effectively in its entirety. Otherwise, a higher coating amount is required. Also, in the second surface treatment step, a coated state causing penetration without overflowing is preferred, but the adjustment of the coating amount is difficult and it is difficult to obtain stable 15 coating over time, over the entire area in the cross-direction and machine-direction.

On the other hand, if the permeability of the substrate exceeds the aforementioned range, the coating liquids to be applied in the first and second surface treatment steps to be 20 explained later show limited permeation, whereby the coating liquid for the ink receiving layer, applied thereon, may become floated by the overflowing of the coating liquid employed in the second surface treatment, or the formed ink receiving layer may generate slight cracks. Also, at the cast 25 step, a satisfactory glossy surface may become difficult to obtain because the evaporation of water or solvent component from the rear surface of the substrate becomes difficult. For similar reasons, it is advantageous to employ a substrate having a Stöckigt sizing degree within a range of 100 to 400 30 seconds and a Bekk smoothness within a range of 100 to 500 seconds. Also, in order to obtain a recording medium comparable in quality to a silver halide photograph, it is preferred to employ a substrate of a basis weight of 160 to 230 g/m<sup>2</sup> and a Gurley stiffness of 7 to 15 mN.

35 In the following there will be explained material for forming the ink receiving layer, to be employed in the embodiment relating to the ink receiving layer.

The ink receiving layer can be formed by applying a coating liquid including a pigment and a binder. It is 40 particularly preferred to include alumina hydrate as a principal component in consideration of dye fixing property, transparency, print density, color forming ability and glossiness, but there can also be employed an inorganic pigment such as light calcium carbonate, heavy calcium carbonate, magnesium carbonate, kaolin, aluminum silicate, diatomaceous earth, calcium silicate, magnesium silicate, synthetic amorphous silica, colloidal silica, alumina, or magnesium hydroxide; or an organic pigment such as styrenic plastic 45 pigments, acrylic plastic pigments, polyethylene particles, microcapsule particles, urea resin particles or melamine resin particles.

As alumina hydrate, there can be advantageously 50 employed a material represented by the following general formula (1):



wherein n represents 0, 1, 2 or 3; m represents a value of 0 to 10, preferably 0 to 5, but m and n are not 0 at the same time. Since mH<sub>2</sub>O represents a cleavable water phase not involved in many cases in the crystal lattice formation, m can be an integral or non-integral value, and may reach 0 when such material is heated.

The alumina hydrate can be produced by a known method such as a hydrolysis of aluminum alkoxide or sodium aluminate as described in U.S. Pat. Nos. 4,242,271 and 4,202,870, or by a neutralization of an aqueous solution of

sodium aluminate etc. with an aqueous solution of aluminum sulfate or aluminum chloride, as described in Japanese Patent Publication No. 57-44605. In the embodiment relating to the ink receiving layer, there is advantageously employed an alumina hydrate showing a boemite structure or an amorphous structure in the X-ray diffraction analysis, particularly that described in Japanese Patent Application Laid-open Nos. 7-232473, 8-132731, 9-66664 and 9-76628.

When executing the cast step by moistening the ink receiving layer by a rewetting method in order to provide the surface of the recording medium with glossiness, it is preferred to employ alumina hydrate of platelet shape with a low orienting tendency. The platelet-shaped alumina hydrate, showing a high water absorption and allowing easy penetration of the rewetting solution, causes the swelling of the ink receiving layer, whereby the alumina hydrate particles can be easily rearranged. It is therefore possible to obtain a high gloss. Also, the production efficiency at the cast step is improved because of the efficient penetration of the rewetting solution.

In the embodiment relating to the ink receiving layer, polyvinyl alcohol is employed as a binder for the coating liquid for forming the ink receiving layer. The content of polyvinyl alcohol is preferably from 5 to 20 mass % with respect to alumina hydrate. Also, an already known binder may be employed in combination with polyvinyl alcohol, as the binder to be used for forming the ink receiving layer in the embodiment relating to the ink receiving layer.

For the formation of the ink receiving layer, it is extremely effective to include at least one substance selected from the group of boric acid and borate salts in the material for forming the ink receiving layer in the above-described manner. The boric acid employable for this purpose is not limited to orthoboric acid ( $H_3BO_3$ ) but also includes metaboric acid and hypoboric acid. The borate salt is preferably a water-soluble salt of boric acid mentioned above, and specific examples include alkali metal salts of boric acid such as sodium salts ( $Na_2B_4O_7 \times 10H_2O$ ,  $NaBO_2 \times 4H_2O$  etc.), or potassium salts ( $K_2B_4O_7 \times 5H_2O$ ,  $KBO_2$  etc.), and ammonium salts of boric acid ( $NH_4B_4O_9 \times 3H_2O$ ,  $NH_4BO_2$  etc.), and alkali earth metal salts such as magnesium salts or calcium salts of boric acid.

It is preferred to employ orthoboric acid in consideration of the stability over time of the coating liquid and the suppression of crack generation. It is also preferably employed within a range of 1.0 to 15.0 mass % in solid boric acid with respect to polyvinyl alcohol in the ink receiving layer. Even within this range, crack generation may take place and a selection of the conditions is therefore necessary. Also, a content exceeding this range deteriorates the stability over time of the coating liquid and is therefore undesirable. More specifically, since the coating liquid is used over a prolonged period in production, a high content of boric acid induces a viscosity increase in the coating liquid or a gelation during such period, thereby frequently requiring a replacement of the coating liquid or a cleaning of the coater head, thus significantly deteriorating the productivity. Also, a content exceeding the aforementioned range tends to generate spot-shaped defects on the surface (cast surface) in the cast process for the same reasons as in the first and second surface treatments to be explained later, whereby a uniform and satisfactory glossy surface may not be obtained.

The ink receiving layer thus formed preferably has pore properties meeting the following conditions, in order to achieve objects and effects of a high ink absorbing property and a high fixing ability. At first, the ink receiving layer preferably has a pore volume within a range of 0.1 to 1.0

$cm^3/g$ . A pore volume less than this range cannot provide a sufficient ink absorbing property, thus providing an ink receiving layer of an inferior ink absorbing property, in which the ink may overflow in certain cases to generate bleeding in the image. On the other hand, a pore volume exceeding this range tends to generate cracks or a powder falling in the ink receiving layer. Also, the ink receiving layer preferably has a BET specific surface area of 20 to 450  $m^2/g$ . If the surface area is less than this range, a sufficient gloss may not be obtained and the image may appear whitish because of increased haze (lowered transparency). Also in such case, the dye absorbability may become undesirably low. On the other hand, a surface area exceeding the above-mentioned range may tend to generate cracks in the ink receiving layer. The pore volume and the BET specific surface area can be determined by a nitrogen adsorption-desorption method.

Also, in forming the ink receiving layer, the producing method according to the embodiment relating to the ink receiving layer can be applied to increase freedom of choice regarding the thickness of the ink receiving layer in comparison with that in the prior technology, namely, to obtain a thicker layer in comparison with the prior technology. In consideration of a high ink absorbing property, there is preferred a dry coating amount of 30 to 50  $g/m^2$ . A coating amount less than such range is undesirable as it cannot provide a sufficient ink absorbing property, resulting in overflow and causing a bleeding phenomenon or resulting in a diffusion of the ink dye even to the substrate, thereby reducing the print density, particularly in a printer employing plural pale-colored inks in addition to three-color inks of cyan, magenta and yellow and a black ink. A coating amount exceeding 30  $g/m^2$  is preferred as it can provide an ink receiving layer showing a satisfactory ink absorbing property even under a high-temperature high-humidity environment, and, at a dry coating amount equal to or less than 50  $g/m^2$ , the coating unevenness decreases in the ink receiving layer which can therefore be produced with a stable thickness.

Boric acid or borate salt to be contained in the coating liquids for the first and second surface treatment steps in the embodiment relating to the ink receiving layer can be similar to that employed in the formation of the ink receiving layer. In consideration of the suppressing effect against crack generation, it is preferred to include borax (sodium tetraborate).

Each of the coating liquids for the ink receiving layer and the surface treatment steps explained in the foregoing is coated using an on-machine or off-machine process so as to obtain an appropriate coating amount mentioned in the foregoing, suitably selecting various coating devices such as a blade coater, a roll coater, an air knife coater, a bar coater, a rod blade coater, a curtain coater, a gravure coater, an extrusion coater, a slide hopper coater or a size press. At the coating operation, it is possible to heat the coating liquid or to heat the coating head for the purpose of viscosity adjustment of the coating liquid.

The drying after coating can be executed by suitably selecting, for example, a hot air dryer such as a straight tunnel dryer, an arch dryer, an air loop dryer or a sinusoidal curve air float dryer, an infrared heating dryer or a microwave dryer.

After the ink receiving layer is formed in the above-described manner, a glossy surface can be formed thereon by a cast process, as will be explained in the following.

The cast process is a method of pressing the ink receiving layer in a moistened state or in a plastic state to a surface of

a heated drum (casting drum) having a mirror surface, and drying the layer in the pressed state thereby transferring the mirror surface to the surface of the ink receiving layer, and is representatively divided into a direct process, a rewetting (indirect) process and a solidification process.

Any of these cast processes can be utilized, but, in the embodiment relating to the ink receiving layer, it is preferred to employ alumina hydrate in the ink receiving layer of the recording medium, and the rewetting cast process is particularly preferred in such case since it can provide a high gloss.

In the producing method for the recording medium in the embodiment relating to the ink receiving layer, it is also possible to add a step of forming a rear layer on the rear surface (opposite to the surface on which the ink receiving layer is formed) of the substrate, thereby producing a recording medium having a rear layer. The formation of the rear layer is effective for reducing a curl generated prior to or after printing.

In consideration of the effect for reducing curling, there is preferred a layer which generates, upon absorbing moisture, a shrinkage similar to that in the undercoat layer and/or the ink receiving layer on the top surface of the substrate, and it is preferred to employ a pigment and a binder similar to those employed in these layers. It is more preferred to employ a pigment and a binder similar to those employed in the thicker ink receiving layer. The rear layer may be formed before or after the first surface treatment, after the formation of the ink receiving layer or after the cast process.

Also, in the case of producing the recording medium of the embodiment relating to the ink receiving layer, it is also possible, if necessary, to provide another layer such as the aforementioned undercoat layer, between the rear layer and the substrate. In such case it is also possible to form a glossy surface on the rear surface, thereby obtaining a recording medium having glossy surfaces on both the front surface and the rear surface. Also, two-sided printing is possible by making it possible to print on the rear layer, or the rear layer and/or the front layer.

Also, in the formation of the rear layer, in order to suppress crack generation as in the ink receiving layer, it is possible to execute the first surface treatment/second surface treatment/rear layer formation on the rear surface of the substrate, namely, to execute the first surface treatment and then the second surface treatment, then to apply a coating liquid for the rear layer while the substrate is maintained in a moist state, and then to dry such coating liquid. However, either one of the first surface treatment and the second surface treatment may be adequate in certain cases (depending on the state of crack generation on the rear layer). FIG. 4 is a schematic cross-sectional view showing a preferred example of the construction of the recording medium produced as explained in the foregoing. The construction includes a base paper 1; an undercoat layer 2 containing a pigment, a binder etc.; an undercoat layer 3; a surface treatment 4 prepared by applying and drying a borax-containing coating liquid; a surface treatment 5 prepared by applying a borax-containing coating liquid; an ink receiving layer 6 (containing alumina hydrate, polyvinyl alcohol, boric acid etc.) prepared by applying and drying a coating liquid while the undercoat layer/base paper is maintained in a moist state due to the surface treatments; and a rear layer 7 including a pigment, a binder etc. The base paper 1 and undercoat layers 2 and 3 constitute a substrate 8.

Referring to FIGS. 2 and 3, a feature of the recording medium is that the ink receiving layer includes a first layer region in which the binder is crosslinked with a first

crosslinking agent and is homogenized relative to the pigment, and a second layer region in which the binder is crosslinked by a second crosslinking agent so as to have a higher crosslinking degree than in the first layer region, and that the first layer region is positioned closer to the ink recording surface than the second layer region. This is a novel recording medium, in which the aforementioned loss of the binder is prevented and pores formed by the pigment aggregated by the crosslinked binder of the higher crosslinking degree are formed stably also in the second layer region, whereby the recorded ink can be adequately absorbed in the ink receiving layer and sharp image formation can be attained without ink diffusion to the surrounding area.

The crosslinking degree in the second layer region substantially intensifies the crosslinking of the binder, so that the dispersion state of the binder at the interface is made uniform, without formation of extremely concentrated areas or extremely deficient areas, thereby preventing unnecessary passage of the binder itself and providing an anchoring effect of the binder if the interface has irregularities. The aforementioned crosslinking degree can be judged by a relative difference in quantity or a ratio thereof of an element common to the first crosslinking agent and the second crosslinking agent (for example boron "B") respectively contained in the first layer region and the second layer region (for example a ratio of five times or higher). Examples of specific materials and a production method are that the recording medium is formed by applying a coating liquid, prepared by mixing and dissolving alumina hydrate as the pigment, polyvinyl alcohol as the binder and orthoboric acid as the first crosslinking agent, on a moist surface containing a tetraborate salt as the second crosslinking agent for forming the second layer region. Also, as a practical example, in such coating liquid the content of orthoboric acid per unit area is less than the content of sodium tetraborate per unit area in the moist surface.

Thus, there is provided a recording medium including an ink receiving layer containing at least a pigment capable of holding the coloring agent of the ink and showing a viscosity change in response to pH, and a binder for the pigment, the recording medium being having the feature that the ink receiving layer includes a first layer region in which the binder is crosslinked with a first crosslinking agent of a pH value capable of maintaining the pigment at a low viscosity, and a second layer region in which the binder is crosslinked by a second crosslinking agent of a pH value capable of maintaining the pigment at a high viscosity, and that the first layer region is positioned closer to the ink recording surface than the second layer region. Based on the relationship of the pigment and the first and second crosslinking agents constituting the ink receiving layer, a pH change is made to provide a high viscosity in the pigment and the second layer is reasonably formed by the binder which is progressively crosslinked by the crosslinking agent. Thus, the formation of the excellent pore distribution and the binder crosslinked without loss enable appropriate absorption of the ink recorded in the ink receiving layer, and the ink and the coloring agent do not diffuse to the surrounding area in the ink receiving layer. This provides sharper image formation. The second layer region, having a larger crosslinking degree due to the second crosslinking agent than in the first layer region, can suppress the swelling of the entire ink receiving layer when the ink is supplied thereto, thus avoiding a change in the image. Such recording medium can be securely produced by a production method wherein the pigment has a low viscosity at a relatively low pH value, but changes to a high viscosity at a relatively high pH value, and

the second layer region is formed by applying a coating liquid of a low pH value, prepared by mixing and dissolving the pigment, the binder and the first crosslinking agent, on a moist surface containing the second crosslinking agent and having a high pH value.

The recording medium wherein the first layer region is positioned closer to the ink recording surface than the second layer region and has a high pH value is similar to the aforementioned second invention, but has an ink receiving layer having pores of uniform size formed by the pigment, utilizing the characteristics of the pigment to achieve binding by the crosslinked binder while accelerating the crosslinking of the binder by the crosslinking agent and the aggregation of the pigment. Thus, the ink receiving layer shows a distribution of permeation that is stable in the direction of its thickness, thereby absorbing the recorded ink more appropriately without diffusion of the ink and the coloring agent to the surrounding area in the ink receiving layer, thus attaining an extremely sharp image formation. Particularly in order to prevent the loss of the binder of the coating liquid into the coated surface side and to achieve efficient removal of the solvent in the coating liquid, utilizing the reaction speed or the reaction state at the liquid-liquid contact interface, it is preferred that the ink receiving layer is formed by applying a coating liquid, prepared by mixing and dissolving at least alumina hydrate as the pigment, polyvinyl alcohol as the binder and orthoboric acid as the first crosslinking agent for forming the first layer region, on a moist surface containing a tetraborate salt as the second crosslinking agent, for forming the second layer region. Also, for obtaining different crosslinking degrees, it is further preferred that the content of orthoboric acid in the coating liquid per unit area is less than the content of sodium tetraborate contained per unit area in the moist surface, or that the pigment is alumina hydrate, the binder is polyvinyl alcohol and the first and second crosslinking agents contain the same boron element "B" wherein the amount of boron "B" contained in the second layer region is two times or more of the amount of boron "B" contained in the first layer region.

The production methods shown in FIGS. 2 and 3 include a step of applying a coating liquid, containing the pigment, the binder and the first crosslinking agent for crosslinking the binder, on a moist surface containing the second crosslinking agent for crosslinking the binder, wherein the crosslinking reaction by the second crosslinking agent at the contact interface between the coating liquid and the moist surface is accelerated in comparison with the crosslinking reaction by the first crosslinking agent in the coating liquid. This utilizes the reaction speed or the reaction state at the aforementioned liquid-liquid contact interface, thereby enabling production of a recording medium of a stable performance, while preventing the loss of the binder of the coating solution into the coated surface side. As a result, there can be formed a first layer region in which the binder is crosslinked by the first crosslinking agent and is made relatively homogeneous with the pigment, and a second layer region in which the binder is crosslinked by the second crosslinking agent so as to have a crosslinking degree higher than in the first layer region. More preferably, in addition to such construction, the aggregation of the pigment can be limited at the same time by a method for producing a recording medium in which the pigment shows a viscosity change in response to pH, wherein the first crosslinking agent provides a pH value capable of maintaining the pigment at a low viscosity, the second crosslinking agent provides a pH value capable of maintaining the pigment at

a high viscosity, and a pH change is generated at the aforementioned contact interface to induce aggregation of the pigment and crosslinking of the binder. In this form, there is realized that the second crosslinking agent is superior in the crosslinking reaction to the first crosslinking agent which is capable of crosslinking the binder, the content of the first crosslinking agent per unit area in the aforementioned coating liquid is smaller than the content of the second crosslinking agent per unit area in the aforementioned moist surface, and the pigment is alumina hydrate, the binder is polyvinyl alcohol, the first crosslinking agent and the second crosslinking agent include the same boron element "B" and the amount of boron "B" contained in the second layer region is twice or more of the amount of boron "B" contained in the first layer region".

In the aforementioned embodiment relating to the ink receiving layer, since it is preferred, at the aforementioned crosslinking reaction, to exclude the liquid component such as the solvent (water in case of PVA (preferably purified water in order to avoid impurity for alumina)) for dissolving the binder of the coating liquid, the recording medium preferably includes, as the substrate for supporting the ink receiving layer, a porous member (paper, pulp, porous layer etc.) into which the liquid component of the coating liquid can permeate. In addition, in order to improve the adhesion and the strength of the ink receiving layer to the substrate (anchoring effect), it is also preferred that the aforementioned wet surface is not a smooth surface, but has recesses for the coating liquid and causes crosslinking of the binder in such recesses.

In the following, the present invention will be further clarified by examples and comparative examples, but the present invention is not limited by such examples. In the following description, "part" and "%" are based on mass unless otherwise specified.

#### EXAMPLE 1

##### Preparation of Substrate

A pulp slurry formed by 67 parts of leaf bleached kraft pulp (LBKP) with a freeness of 450 ml CSF (Canadian Standard Freeness), and 8 parts of needle bleached kraft pulp (NBKP) with freeness of 480 ml CSF was added with 0.4 parts of a paper strengthening agent (RB-151, manufactured by Harima Chemicals Co.) and 2 parts of aluminum sulfate and was adjusted to a pH value of 7.8, and a substrate was prepared.

##### Cationizing Treatment of Substrate

The obtained substrate was treated, on a surface on which an ink receiving layer was to be formed, with a cationic resin having a benzyl group and obtained in the following manner, so as to obtain an applied amount of 1 g/m<sup>2</sup> after drying. The cationic resin was obtained by dissolving 50.6 g of a 60% aqueous solution of methacryloyloxyethyl dimethylbenzylammonium chloride and 2.22 g of a 40% aqueous solution of acrylamide in 140 g of ion-exchanged water, then heating to 70° C. under nitrogen blowing, adding 10 g of a 0.1% aqueous solution of 2,2'-azobis(2-aminodipropylene)hydrochloride and executing a reaction for 2 hours at 85° C.

##### Preparation of Coating Liquid for Undercoat Layer

On both sides of the substrate subjected to the aforementioned cationizing treatment, undercoat layers were formed with a coating liquid prepared in the following manner. A slurry with a solid concentration of 70%, containing 100 parts by mass of a filler formed by kaolin (Ultra White 90,

manufactured by Engelhard Ltd.)/zinc oxide/aluminum hydroxide with a weight ratio of 65/10/25 and 0.1 parts by mass of a commercially available polyacrylic acid-based dispersant, was added with 7 parts by mass of a commercially available styrene-butadiene latex and was adjusted to a solid content of 60% to obtain a coating liquid for the undercoat layer.

#### Coating of Coating Liquid for Undercoat Layer

The coating liquid obtained above was applied with a blade coater on both sides of the substrate so as to obtain a dry coating amount of 15 g/m<sup>2</sup> and was dried. Then a machine calender finishing (linear pressure 150 kgf/cm) was applied to obtain a substrate with a basis weight of 185 g/m<sup>2</sup>, a Stöckigt sizing degree of 300 seconds, an air permeability of 3000 seconds and a Bekk smoothness of 180 seconds. This substrate was subjected to a cationizing treatment on one side with an undercoat layer thereon, and had the undercoat layers on both sides.

#### Surface Treatment of Undercoat Layer

The undercoat layer prepared as explained in the foregoing was subjected to a first surface treatment in the following manner. A coating liquid employed for the first surface treatment was a 5% aqueous solution of borax, heated to 30° C. This coating liquid was applied with a gravure coater on the undercoat layer at a speed of 60 m/min so as to obtain a dry coating amount of 0.4 g/m<sup>2</sup>, and was then dried at 60° C.

Then the undercoat layer after the first surface treatment was subjected to a second surface treatment. The second surface treatment was executed by employing the same 5% borax aqueous solution heated to 30° C. as in the first surface treatment as a coating liquid and applying such coating liquid with an air knife coater at a speed of 30 m/min so as to obtain a wet coating amount of 10 g/m<sup>2</sup> (corresponding to a dry coating amount of 0.5 g/m<sup>2</sup>). This coating amount, under visual observation, was such that the coating liquid did not overflow on the undercoat layer but just impregnated therein.

#### Preparation of Coating Liquid for Ink Receiving Layer

After the application of the coating liquid in the aforementioned second surface treatment, namely in a state in which the undercoat layer has been just impregnated with the coating liquid, an ink receiving layer was formed on the undercoat layer in the following manner.

At first, a coating liquid for forming the ink receiving layer was prepared by the following procedure. Disperal HP13 (manufactured by Sasol Co.) as alumina hydrate A was dispersed in purified water so as to obtain a solid content of 5 mass %, and the dispersion was adjusted to pH 4 with an addition of hydrochloric acid and agitated for a while. Then the dispersion was heated to 95° C. under agitation and was maintained at this temperature for 4 hours. The dispersion, while maintained at this temperature, was adjusted to pH 10 with sodium hydroxide, agitated for 10 hours, then returned to room temperature and adjusted to a pH value of 7 to 8. It was then subjected to a desalting process and was deflocculated with an addition of acetic acid to obtain a colloidal sol. Alumina hydrate B, obtained by drying the colloidal sol, showed a boemite structure (pseudo boemite) in an X-ray diffraction analysis. It also showed a BET specific surface area of 143 g/m<sup>2</sup> and a pore volume of 0.8 cm<sup>3</sup>/g. In an electron microscopic observation, it had a platelet shape with an average aspect ratio of 7.5 and a squareness of 0.7.

Separately, polyvinyl alcohol PVA117 (manufactured by Kuraray Inc.) was dissolved in purified water to obtain an aqueous solution of a solid content of 9 mass %. The colloidal sol of alumina hydrate B, obtained above, was concentrated to obtain a dispersion of 22.5 mass %, and a 3% aqueous solution of boric acid was added in such a manner that the boric acid solid corresponded to 0.50 mass % of the solid of alumina hydrate B. The thus-obtained alumina hydrate dispersion containing boric acid and the separately prepared aqueous solution of polyvinyl alcohol were mixed with a static mixer so as to obtain a ratio of 100:8 with respect to the alumina hydrate solid and the polyvinyl alcohol solid, thereby obtaining a coating liquid for the ink receiving layer.

#### Application of Coating Liquid for Ink Receiving Layer

The coating liquid for the ink receiving layer prepared as explained above, in a state immediately after the mixing of the alumina hydrate dispersion containing boric acid and the aqueous solution of polyvinyl alcohol, was applied with a die coater, on the undercoat layer of the side subjected to the cationizing treatment, with a speed of 30 m/min so as to obtain a dry coating amount of 35 g/m<sup>2</sup> and was dried at 170° C. to form an ink receiving layer.

#### Formation of Rear Layer

Also, a rear layer was formed in the following manner, on the undercoat layer on a side of the substrate opposite to the ink receiving layer. Alumina hydrate Disperal HP 13/2 (manufactured by Sasol Inc.) was dispersed in purified water so as to obtain a solid content of 18 mass %, and was then subjected to a centrifuging process. This dispersion and the same aqueous solution of polyvinyl alcohol as that employed in forming the ink receiving layer were mixed with a static mixer so as to obtain a ratio of 100:9 between the alumina hydrate solid and the polyvinyl alcohol solid, and the mixture was immediately applied with a die coater at a speed of 35 m/min so as to obtain a dry coating amount of 23 g/m<sup>2</sup>, thereby forming a rear layer.

#### Formation of Glossy Surface

On the coated base paper (substrate) on which the ink receiving layer and the rear layer were formed as explained above, a glossy surface was formed in the following manner on the surface of the ink receiving layer. At first, for executing a rewetting cast process, water as a rewetting solution was uniformly applied to the aforementioned base paper to moisten at least the ink receiving layer. Then, in such moistened state, it was pressed to a cast drum heated to 100° C. and having a mirror surface and dried at a speed of 30 m/min, thereby obtaining a recording medium for ink of the present example, having a glossy surface on one side. This was regarded as a recording medium 1 for ink. A measurement of "N" distribution on a cross section thereof provided a distribution shown in FIG. 1.

#### EXAMPLE 2

A recording medium 2 for ink was prepared in the same manner as in Example 1, except that the cationizing treatment was so executed as to obtain a dry applied amount of 3 g/m<sup>2</sup>.

#### EXAMPLE 3

A recording medium 3 for ink was prepared in the same manner as in Example 1, except that the cationizing treatment was so executed as to obtain a dry applied amount of 5 g/m<sup>2</sup>.

#### EXAMPLE 4

A recording medium **4** for ink was prepared in the same manner as in Example 1, except that the cationizing treatment was so executed as to obtain a dry applied amount of 0.5 g/m<sup>2</sup>.

### EXAMPLE 5

A recording medium **5** for ink was prepared in the same manner as in Example 1, except that the cationizing treatment was so executed as to obtain a dry applied amount of 0.2 g/m<sup>2</sup>.

### EXAMPLE 6

A recording medium 6 for ink was prepared in the same manner as in Example 1, except that the cationizing treatment was executed with a cationic resin (trade name: Sanfix PAC-700 conc., manufactured by Sanyo Chemical Industries Co.).

### COMPARATIVE EXAMPLE 1

A recording medium 7 for ink was prepared in the same manner as in Example 1, except that the cationizing treatment was not executed.

### COMPARATIVE EXAMPLE 2

A recording medium 8 for ink was prepared in the same manner as in Example 1, except that the cationizing treatment was not executed, and that the cationic resin employed for the cationizing treatment in Example 2 was mixed in the coating liquid for the undercoat layer so as to obtain a solid ratio (cationic resin/undercoat layer solid matter) of 5/100.

### COMPARATIVE EXAMPLE 3

The cationizing treatment was not executed, and the cationic resin employed for the cationizing treatment in Example 2 was mixed in the coating liquid for the ink receiving layer so as to obtain a solid ratio (cationic resin/undercoat layer solid matter) of 5/100. However, the coating liquid for the ink receiving layer caused gelation and coagulation, so that the ink recording medium could not be prepared.

## Evaluation

The recording media for ink 1 to 8, obtained in the foregoing Examples and Comparative Examples, were evaluated by the following methods and criteria. Obtained results of evaluation are summarized in Table 1.

## Surface Property

Presence (yes) or absence (none) of crack generation on the surface of the ink receiving layer was confirmed by visual observation.

## Mirror Surface Glossiness

A mirror surface glossiness was measured at 20° and 75°, by a gloss measuring meter (trade name: VG2000, manufactured by Nihon Denshoku Kogyo Co.).

## 15 Moisture Resistance 1 of Image

White characters “○△□” were printed on a solid blue area (cyan 100%+magenta 100%) formed on each of the recording media for ink 1 to 8 with BJF900 (trade name, manufactured by Canon Inc.), and the obtained print was allowed to stand for 7 days in an environment of 23°C./80% humidity. After the standing, a state showing remaining white characters was evaluated as rank A, a state with illegible white characters was evaluated as rank C, and an intermediate state was evaluated as rank B.

## <sup>25</sup> Moisture Resistance 2 of Image

An evaluation was made using the same method and the same criteria as in the above moisture resistance 1, except that the ink recording medium after image formation was allowed to stand in an environment of 30°C./80% humidity.

### 30 Light Fastness of Image

On each of the recording media for ink 1 to 8, 100% print areas of black, cyan, magenta and yellow of 3 cm square each were printed with BJF900 (trade name, manufactured by Canon Inc.), and the obtained print was subjected to an accelerated deterioration test with a light fastness tester (trade name: Ci-4000, manufactured by Atlas Electric Device Company). The light fastness tester was set at conditions of a black panel temperature: 55°C., an illumination intensity: 0.39 W/m<sup>2</sup>, an in-chamber temperature: 45°C., an in-chamber humidity: 60% RH, and a test period of 24 hours. The image density of the print was measured before and after the light fastness test and the retention rate was calculated as follows. The image density was measured with a Macbeth densitometer (trade name: RD-918, manufactured by Kollmorgen Corporation):

Retention rate(%)=(image density after test)/(image density before test)×100

TABLE 1

TABLE 1-continued

| Surface     | <u>Results of evaluation</u> |                             |     |                         |                         |                                   |      |         |
|-------------|------------------------------|-----------------------------|-----|-------------------------|-------------------------|-----------------------------------|------|---------|
|             | property                     | Mirror surface glossi- ness |     | Moisture resis- tance 1 | Moisture resis- tance 2 | Light fastness (retention rate %) |      |         |
|             |                              | 20°                         | 75° |                         |                         | black                             | cyan | magenta |
| Comp. Ex. 2 | none                         | 25                          | 65  | B                       | B                       | 77                                | 93   | 74      |
| Comp. Ex. 3 | —                            | —                           | —   | —                       | —                       | —                                 | —    | 78      |

15

The amount of boron "B" in the first layer region was  $2.61 \times 10^{-3}$  mol/m<sup>2</sup>, while that in the second layer region was  $9.94 \times 10^{-3}$  mol/m<sup>2</sup>, so that the amount of boron "B" in the second layer region was 3.8 times that in the first layer region. In the present examples, there is required a quantitative relationship of 2 times or higher.

The amount of boron "B" contained in the first layer region was calculated by the following formulas:

$$\begin{aligned} & \text{(dry coating amount of ink receiving layer: } 35) \times \\ & \quad (\text{amount of boric acid: } 22.5 \times 0.5\%) / (\text{amount of boric acid: } 22.5 \times 0.5\%) + (\text{amount of PVA: } 22.5 \times \\ & \quad 8/100) + (\text{amount of alumina hydrate: } 22.5) \} = 0.16 \text{ g/m}^2 \end{aligned}$$

$$0.16 / (\text{molecular weight of boric acid: } 61.8) = 2.61 \times 10^{-3} \text{ mol/m}^2.$$

Also, the amount of boron "B" contained in the second layer region was calculated by the following formula:

$$\begin{aligned} & \text{(dry coating amount of second surface treatment: } 0.5) / (\text{molecular weight of borax: } 201.2) \times (\text{mo-} \\ & \quad \text{lar amount of B per 1 mole of borax: } 4) = 9.94 \times 10^{-3} \text{ mol/m}^2. \end{aligned}$$

In the foregoing, the molecular weight of borax was calculated for Na<sub>2</sub>B<sub>4</sub>O<sub>7</sub> since borax was in an impregnated state in the undercoat layer and not in a dried state.

As will be apparent from the foregoing examples, the borax salt is superior in the crosslinking property to orthoboric acid, and is different in quantity even after drying. Also, alumina hydrate used as a pigment shows a rapid viscosity change at about pH 7, showing a low viscosity at the acidic side and a high viscosity at the alkaline side. Also, an aqueous solution of the borax salt is alkaline, while an aqueous solution of orthoboric acid is acidic. Besides, the coating liquid for forming the ink receiving layer is acidic and dissolves alumina hydrate while the reaction at the aforementioned liquid-liquid interface changes at about pH 7, so that the crosslinking reaction of PVA securely takes place and the alumina hydrate causes a viscosity increase and aggregation whereby water (preferably purified water for preventing impurity for alumina) as the solvent is separated from the PVA serving as the binder, and penetrates into the substrate. A pH measurement on a cross section of the prepared ink receiving layer showed a pH value of 6.2 to 6.4 in the first layer region (for example, at the surface) in the embodiment relating to the ink receiving layer, and a pH value of about 6.8 in the second layer region. Thus, the examples shown above demonstrate the inventions in the embodiment relating to the ink receiving layer and exhibit the effects thereof.

The effect of the embodiment relating to the ink receiving layer can be further enhanced when applied to a recording

medium for recording ink droplets as an image, to a recording head or to a recording apparatus of a bubble jet method among the ink jet recording methods.

As to its representative configuration and principle, for example the one practiced by the use of the basic principle disclosed in U.S. Pat. Nos. 4,723,129 and 4,740,796 is preferred. This system is applicable to either of the so-called on-demand type and the continuous type. Particularly, the case of the on-demand type is effective because, by applying at least one driving signal which gives rapid temperature elevation exceeding nucleus boiling corresponding to the recording information on an electrothermal converting member arranged corresponding to the sheets or liquid channels holding ink, thermal energy is generated at the electrothermal converting member to induce film boiling at the heat action surface of the printing head, and a bubble can be consequently formed in the ink in one-to-one response to the driving signals. By discharging the ink through a discharge aperture by the growth and shrinkage of the bubble, at least a droplet is formed. By forming the driving signals into pulse shapes, growth and shrinkage of the bubble can be effected instantly and adequately to accomplish more preferable discharging of the ink so as to have particularly excellent response characteristics. As for the driving signals of such pulse shapes, those disclosed in U.S. Pat. Nos. 4,463,359 and 4,345,262 are suitable. Further excellent recording can be performed by employment of the conditions described in U.S. Pat. No. 4,313,124 of the invention concerning the temperature elevation rate of the above-mentioned heat action surface.

#### POSSIBILITY OF INDUSTRIAL APPLICATION

As explained in the foregoing, the present invention provides an ink recording medium able to absorb a large amount of ink at a high speed, excellent in color forming property and capable of forming a high quality image, and a production method for such ink recording medium. In particular, the present invention provides an ink recording medium capable of suppressing image deterioration due to dye displacement, which tends to take place when the image is maintained in a high humidity condition, and image deterioration due to light when the image is displayed, and excellent in stability over time of the printed image, and a production method for such ink recording medium.

What is claimed is:

1. A recording medium for ink comprising a substrate, an undercoat layer and a porous ink receiving layer provided in this order, wherein said undercoat layer comprises an increasing region in which a reactive substance capable of reacting

## 31

with a coloring agent contained in ink and holding said coloring agent is present with such a distribution as to increase in the direction of depth of said undercoat layer, and a position with the maximum concentration of the reactive substance is in the increasing region.

2. A recording medium for ink according to claim 1, wherein said increasing region is not present in said ink receiving layer.

3. A recording medium for ink according to claim 2, wherein said ink receiving layer contains alumina hydrate and a binder for said alumina hydrate.

4. A recording medium for ink according to claim 1, wherein said ink receiving layer contains at least a pigment for holding a coloring agent of an ink, and a binder for said pigment, and said ink receiving layer includes a first layer region in which said binder is crosslinked with a first crosslinking agent and is made uniform relative to said pigment and a second layer region in which said binder is crosslinked with the first crosslinking agent and a second crosslinking agent so as to have a crosslinking degree higher than that in the first layer region, and said first layer region is positioned closer to said ink recording surface than said second layer region.

5. A recording medium for ink according to claim 4, wherein said ink receiving layer is formed by applying a coating liquid which is formed by mixing and dissolving at least alumina hydrate as said pigment for forming the first layer region, polyvinyl alcohol as said binder and orthoboric acid as said first crosslinking agent, on a moist surface containing a tetraborate salt as said second crosslinking agent for forming said second layer region.

6. A recording medium for ink according to claim 5, wherein the content of said orthoboric acid contained in said coating liquid per unit area is less than a content of said sodium tetraborate contained in said moist surface per unit area.

7. A recording medium for ink according to claim 4, wherein said ink receiving layer is 30 g/m<sup>2</sup> or higher.

8. A recording medium for ink according to claim 1, wherein said ink receiving layer contains at least a pigment for holding a coloring agent of an ink and showing a viscosity change in response to pH, and a binder for said pigment, said ink receiving layer includes a first layer region in which said binder is crosslinked with a first crosslinking agent of a pH value capable of maintaining said pigment at a low viscosity, and a second layer region in which said

## 32

binder is crosslinked with the first crosslinking agent and a second crosslinking agent of a pH value capable of maintaining said pigment at a high viscosity, and said first layer region is positioned closer to said ink recording surface than said second layer region.

9. A recording medium for ink according to claim 8, wherein said second layer region has a crosslinking degree, due to said second crosslinking agent, higher than said first layer region.

10. A recording medium for ink according to claim 8, wherein said pigment has a low viscosity at a relatively low pH value and changes to a high viscosity at a relatively high pH value, and said second layer region is formed by applying a coating liquid of a low pH value, prepared by mixing and dissolving said pigment, said binder and said first crosslinking agent, on a moist surface of a high pH value containing said second crosslinking agent.

11. A recording medium for ink according to claim 1, wherein said ink receiving layer contains at least a pigment capable of holding a coloring agent of an ink and showing a low viscosity at a relatively low pH value and a high viscosity at a relatively high pH value, and a binder for said pigment, said ink receiving layer includes a first layer region in which said binder is crosslinked with a first crosslinking agent of a pH value capable of maintaining said pigment at a low viscosity, and a second layer region in which said binder is crosslinked with the first crosslinking agent and a second crosslinking agent of a pH value capable of maintaining said pigment at a high viscosity, and said first layer region is positioned closer to said ink recording surface than said second layer region and has a higher pH value.

12. A recording medium for ink according to claim 1, wherein said undercoat layer comprises a decreasing region, in which said reactive substance is present in a such distribution as to decrease in the direction of depth of said undercoat layer.

13. A recording medium for ink according to claim 1, wherein said reactive substance is a cationic substance.

14. A recording medium for ink according to claim 13, wherein said cationic substance is not present in said ink receiving layer.

15. A recording medium for ink according to claim 1, wherein said ink receiving layer contains alumina hydrate and a binder for said alumina hydrate.

\* \* \* \* \*

UNITED STATES PATENT AND TRADEMARK OFFICE  
**CERTIFICATE OF CORRECTION**

PATENT NO. : 7,255,901 B2  
APPLICATION NO. : 10/678143  
DATED : August 14, 2007  
INVENTOR(S) : Kenichi Yamaguchi et al.

Page 1 of 2

It is certified that error appears in the above-identified patent and that said Letters Patent is hereby corrected as shown below:

COLUMN 3

Line 4, "printability etc." should read --printability, etc.,"--.

COLUMN 4

Line 38, "outemost" should read --outermost--.

COLUMN 6

Line 30, "alcohol" should read --alcohol,--.

COLUMN 11

Line 29, "of" should read --or--.

COLUMN 12

Line 67, "porous layer" should read --porous layer,--.

COLUMN 13

Line 60, "porous layer" should read --porous layer,--.

COLUMN 17

Line 4, "agent" should read --agent,--.

Line 32, "alcohol" should read --alcohol,--.

Line 43, "defect" should read --defect,--.

COLUMN 19

Line 1, "aluminate etc." should read --aluminate, etc.,--.

Line 38, "NaBO<sub>2</sub>×4H<sub>2</sub>O" should read --NaBO<sub>2</sub>×4H<sub>2</sub>O,--.

Line 39, "KBO<sub>2</sub>" should read --KBO<sub>2</sub>,--.

Line 40, "NH<sub>4</sub>BO<sub>2</sub>" should read --NH<sub>4</sub>BO<sub>2</sub>,--.

UNITED STATES PATENT AND TRADEMARK OFFICE  
**CERTIFICATE OF CORRECTION**

PATENT NO. : 7,255,901 B2  
APPLICATION NO. : 10/678143  
DATED : August 14, 2007  
INVENTOR(S) : Kenichi Yamaguchi et al.

Page 2 of 2

It is certified that error appears in the above-identified patent and that said Letters Patent is hereby corrected as shown below:

COLUMN 21

Line 60, "acid" should read --acid,--.

Line 63, "binder" should read --binder,--.

COLUMN 24

Line 15, "region" should read --region,--.

Line 23, "porous layer" should read --porous layer,--.

COLUMN 30

Line 63, "ink ¶" should read --ink--.

COLUMN 32

Line 34, "a such" should read --such a--.

Signed and Sealed this

Twenty-seventh Day of May, 2008



JON W. DUDAS  
*Director of the United States Patent and Trademark Office*